

## UNITED STATES PATENT OFFICE

2,339,898

## LUBRICANT

Claron N. White, Chicago, Ill., and Frederick H. McLaren, Munster, Ind., assignors to Standard Oil Company, Chicago, Ill., a corporation of Indiana

No Drawing. Application June 30, 1941,  
Serial No. 400,460

6 Claims. (Cl. 196—151)

The present invention relates to lubricants having a high viscosity index, a low pour point and a high viscosity.

The lubrication of certain engines, machines and mechanical devices requires lubricants having special properties among which may be listed high viscosity, high viscosity index and low pour point. Lubricants having these special properties are particularly useful in lubricating gears of various kinds such as rear axles, transmissions and the like. Refined mineral lubricating oils will usually fulfill one or two or the above-mentioned requirements but seldom all three. It has been found, in fact, that a mineral oil having a high viscosity index usually does not have a low pour point.

It is therefore an object of the present invention to provide a lubricant which will have both a high viscosity index and a low pour point.

A further object of the present invention is to provide a mineral lubricating oil having a component which will greatly improve the viscosity index, lower the pour point and at the same time greatly increase the viscosity of the lubricant.

According to the present invention the lubricating composition contains a petroleum oil and a high molecular weight hydrocarbon oil. The latter component, because of its high molecular weight, appearance and physical characteristics is sometimes referred to as a "resin" or a "resinous oil," even though its chemical characteristics are far different from those materials more commonly and more properly known as resins. In order to distinguish the high molecular weight oil more clearly from the comparatively light petroleum oil in the following description, the former will be referred to hereinafter as a resin-like oil.

While light petroleum oils of differing characteristics may be used, depending on the nature and properties desired in the final product, it has been found that from about 60% to about 99% of an oil having a viscosity of from about 50 seconds Saybolt Universal at 100° F. to about 1500 seconds Saybolt Universal at 100° F. and a viscosity index of less than 70 is suitable.

The resin-like oil has a molecular weight of from 1000 to about 2000 and may be added to the oil in quantities ranging from about 1% to about 40% but preferably from about 10% to about 30%. This resin-like oil may be obtained preferably from a Pennsylvania cylinder stock which has been dewaxed at about -40° F. The dewaxed stock is then treated with 4 to 10 volumes of propane at a temperature from about 160° F. to about 180° F. to produce two phases, a lighter propane-soluble phase and a heavy propane-insoluble phase containing the resin-like oils. The heavy fraction is then treated with additional propane at from 135° F. to 170° F., usually about 145° F., the ratio of propane to heavy oil being from about

5 to 1 to about 10 to 1, and usually from about 7 to 1. By this treatment about 3% to about 3½% of the resin-like oil based on the original amount of dewaxed oil precipitates out from the propane-soluble constituents of the dewaxed oil. Although liquefied propane has been referred to as the refining agent, it will be understood that the propane may contain or be replaced by other liquefied normally gaseous hydrocarbons, particularly ethane, isobutane, butane, propylene, butylene, etc. This resin-like oil is a substantially wax-free and asphalt-free product having a Saybolt Universal viscosity at 210° F. of from about 1000 to about 4000 or more seconds, a viscosity index of about 90 or more and a relatively high pour point.

A resin-like oil having suitable characteristics, similar to the foregoing may be obtained from a mixed base oil such as Mid-Continent crude oil. Obviously, in this case, it would be necessary to deasphalt as well as dewax the oil before precipitation of the resin-like oil. When a Mid-Continent oil is used the asphalt may be removed by treatment with propane at temperatures of from 105° F. to 115° F., the oil-propane ratio being about 1 to 2.

A more detailed description of the process for obtaining the resin-like oil will be found in U. S. Patents 2,143,872 and 2,143,882.

It is, of course, very often desirable to improve the extreme pressure properties of the lubricant as well as minimize the corrosive effect of the oil on various metals. To obtain these additional properties various extreme pressure agents and various corrosion inhibitors may be added to the oil in suitable amounts. Chlorine-containing and sulfur-containing extreme pressure agents may be added, such as for example, chlorinated wax, chloralkyl phosphites, salts of chlorinated alkylated aromatic acids, sulfurized sperm oil, sulfurized fatty oils, dibenzyl disulfide, alkyl sulfides, alkyl xanthates and the like. Lead naphthenate, triethanolamine, cyclohexylamine, alkyl phosphates, alkyl phosphites and the like may be added as corrosion inhibitors. Obviously, the extreme pressure agent and corrosion inhibitor, if desired, should be selected, according to the type of service to which the lubricant is to be put. Also, various well-known viscosity index improvers such as high molecular weight olefin polymers, methacrylic polymers and esters may be added if desired, although the resin-like oil is usually sufficient for most purposes. The improved lubricant comprising a light petroleum oil and the resin-like oil may be used with or without extreme pressure additives in the compounding of greases.

In Table I the characteristics of compositions containing various proportions of the resin-like oil and mineral lubricating oil are given.

Table I

| Composition        | Viscosity at 100° F. | Viscosity at 210° F. | Viscosity index | Pour point °F. |
|--------------------|----------------------|----------------------|-----------------|----------------|
| 70% No. 1 oil      |                      |                      |                 |                |
| 30% resin-like oil | 1,103                | 90.6                 | 90.8            | -10            |
| 70% No. 2 oil      | 1,277                | 91.5                 | 77.8            | -15            |
| 30% resin-like oil |                      |                      |                 |                |
| 65% No. 2 oil      | 1,742                | 109.7                | 79.1            | -5             |
| 35% resin-like oil |                      |                      |                 |                |
| 52.5% No. 1 oil    | 1,142                | 90.9                 | 88.1            | -15            |
| 17.5% No. 2 oil    |                      |                      |                 |                |
| 30% resin-like oil |                      |                      |                 |                |
| 35% No. 1 oil      | 1,184                | 91.1                 | 84.9            | -15            |
| 35% No. 2 oil      |                      |                      |                 |                |
| 30% resin-like oil |                      |                      |                 |                |

In Table II the characteristics of oil No. 1 and oil No. 2 as well as the characteristics of the resin-like oil are given:

Table II

| Composition    | Viscosity at 100° F. | Viscosity at 210° F. | Viscosity index | Pour point °F. |
|----------------|----------------------|----------------------|-----------------|----------------|
| No. 1 oil      | 205                  | 44.9                 | 65.3            | 0              |
| No. 2 oil      | 229                  | 45.1                 | 43.3            | -5             |
| Resin-like oil | 2,910                | 195                  | 195             | +80            |

<sup>1</sup> Calculated.

By comparing Tables I and II it will be noted that the pour point of the oil Nos. 1 and 2 are lowered, while the viscosity and viscosity index are raised when the resin-like oil is added to the base oil.

An example of a lubricant having the various improved properties mentioned hereinbefore can be composed of

|                                                   | Per cent |
|---------------------------------------------------|----------|
| No. 1 oil                                         | 50.5     |
| No. 2 oil                                         | 17       |
| Resin-like oil                                    | 29       |
| Chlorinated paraffin wax (extreme pressure agent) | 3        |
| Lead naphthenate (corrosion inhibitor)            | 0.5      |

The characteristics of the above lubricant are given in the following Table III:

Table III

|                                        |       |     |
|----------------------------------------|-------|-----|
| Flash                                  | °F.   | 390 |
| Pour                                   | °F.   | -10 |
| Moisture                               | Trace |     |
| Saybolt Universal viscosity at 100° F. | 1,180 |     |
| Saybolt Universal viscosity at 210° F. | 91.3  |     |
| Viscosity index                        | 85.6  |     |
| Non-combustible sediment per cent      | 0.012 |     |
| Cu. strip (24 hrs. at 200° F.)         |       |     |

No stain or discoloration  
Stability (100 hrs. at 200° F.) test: vis. increase per cent 2.2

Another example of a lubricant which exhibits the desired advantages consists of

|                                                                  | Per cent |
|------------------------------------------------------------------|----------|
| No. 1 oil                                                        | 35       |
| No. 2 oil                                                        | 34.5     |
| Resin-like oil                                                   | 25.5     |
| Chlorinated paraffin wax (extreme pressure agent)                | 3.0      |
| Lead naphthenate (corrosion inhibitor)                           | 0.5      |
| High molecular weight olefin polymers (viscosity index improver) | 1.5      |

Although the present invention has been described with reference to specific examples, these are not to be construed as limitations. The scope of the present invention is defined only by the appended claims.

We claim:

1. A lubricant containing chiefly a mineral lubricating oil having a relatively low viscosity index and a viscosity of from about 50 to about 1500 seconds Saybolt Universal at 100° F. and from about 1% to about 40% of a resin-like oil obtained by treating a substantially asphalt-free, wax-free, lubricating oil stock to effect a separation of a light fraction and a heavy fraction containing the resin-like oil and precipitating the resin-like oil from said heavy fraction by treating said heavy fraction with at least 5 volumes of a liquefied normally gaseous hydrocarbon to precipitate a resin-like oil having a viscosity of from about 1000 to about 4000 seconds Saybolt Universal at 210° F.
2. A lubricant containing from about 60% to about 99% of a mineral lubricating oil having a viscosity index below 70 and a viscosity of from about 50 to about 1500 seconds Saybolt Universal at 100° F. and from about 1% to about 40% of a resin-like oil obtained by treating a substantially asphalt-free, wax-free lubricating oil stock with a liquefied normally gaseous hydrocarbon to effect a phase separation of a light fraction soluble in said liquefied hydrocarbon and a heavy fraction containing the resin-like oil insoluble in said liquefied hydrocarbon, and precipitating the resin-like oil from said heavy fraction by treating said heavy fraction with at least 5 volumes of a liquefied normally gaseous hydrocarbon to precipitate a resin-like oil having a viscosity of from about 1000 to about 4000 seconds Saybolt Universal at 210° F.
3. A lubricant having a high viscosity index and low pour point containing chiefly a mineral lubricating oil having a viscosity index of less than 70 and from about 10% to about 30% of a resin-like oil obtained by treating a substantially asphalt-free, wax-free lubricating oil stock with a liquefied normally gaseous hydrocarbon to effect a phase separation of a light fraction soluble in said liquefied hydrocarbon and a heavy fraction containing the resin-like oil insoluble in said liquefied hydrocarbon, and precipitating the resin-like oil from said heavy fraction by treating said heavy fraction with at least 5 volumes of the liquefied normally gaseous hydrocarbon to precipitate a resin-like oil having a viscosity from about 1000 to about 4000 seconds Saybolt Universal at 210° F.
4. A lubricant having a high viscosity index and a low pour point containing from about 60% to about 99% of a mineral lubricating oil having a viscosity index below 70 and a viscosity of from about 50 to about 1500 seconds Saybolt Universal at 100° F. and from about 1% to about 40% of a resin-like oil obtained by treating a substantially asphalt-free, wax-free lubricating oil stock with from about 4 to about 10 volumes of a liquefied normally gaseous hydrocarbon to effect a phase separation of a light fraction soluble in said liquefied hydrocarbon and a heavy fraction containing the resin-like oil insoluble in said liquefied hydrocarbon, and precipitating the resin-like oil from said heavy fraction by treating said heavy fraction with from about 5 to about 10 volumes of said liquefied normally gaseous hydrocarbon.
5. A method for improving the viscosity index and lowering the pour point of a mineral oil comprising incorporating therewith a minor amount of a resin-like oil obtained by treating a substantially asphalt-free, wax-free lubricating oil stock to effect a phase separation of a light fraction and a heavy fraction containing the resin-

like oil, and precipitating the resin-like oil from said heavy fraction by treating said heavy fraction with at least 5 volumes of a liquefied normally gaseous hydrocarbon to precipitate a resin-like oil having a viscosity from about 1000 to about 4000 seconds Saybolt Universal at 210° F.

6. A lubricant as claimed in claim 1 wherein

the mineral lubricating oil component has a low pour point and the resin-like oil has a pour point higher than said mineral lubricating oil component, said lubricant having a pour point at least as low as said mineral lubricating oil component.

CLARON N. WHITE.  
FREDERICK H. MACLAREN.